

2,965,931

**IMPROVED METHOD FOR PRESSURE BAKING OF CARBON ARTICLES**

**Lorne B. Alden and Frank P. Holloway, Fostoria, Ohio, assignors to Union Carbide Corporation, a corporation of New York**

**No Drawing. Filed Oct. 24, 1957, Ser. No. 692,034**

**2 Claims. (Cl. 18—47.5)**

This invention relates to the use of a sulfur-containing mix in the production of shaped carbon articles by pressure baking.

A recently developed pressure baking method for producing carbon articles comprises confining in a refractory lined mold, a mixture of finely divided carbonaceous particles with a fusible and carbonizable carbonaceous binder susceptible of thermal decomposition subjecting the mixture within the mold to a high mechanical pressure of the order of 4500 pounds per square inch to compress the same, and passing an electrical current of about 500 amperes per square inch of compressed mixture in the mold to heat the mixture to a temperature at which substantially complete carbonizing of the binder constituent occurs. By means of this process, it is possible to produce in about eight minutes carbon articles which heretofore required a production time of eight weeks.

In the above-described process, pitch and certain other binder materials produce volatile substances which condense on the press, punches, and cold sections of the mold. Accumulation of such substances prevents or interferes with proper operation of the equipment, and in extreme case can occasion minor explosions.

The main object of the present invention, therefore, is to provide means for preventing the accumulation of condensed volatile material on carbon-baking equipment employed in the process described.

This object is achieved in accordance with the present invention, which is based upon the unpredictable discovery that the addition of finely divided sulfur to the binder material or "green" unbaked mix results in reactions which, at the process temperature, slightly increase the deposition of binder carbon and more characteristically, produce largely non-condensing volatile gases, thereby avoiding the accumulation of unwanted material on the equipment.

In the practice of the invention, sulfur is added in a quantity ranging from 3 to 20 percent by weight of the pitch binder.

Sulfur cannot be used with all carbonaceous binders, but only with those having a softening point less than 300° C., such binders hereafter being denominated "sulfur-reactive binders." This temperature limits allows the binder to be melted and distributed in the carbon aggregate before the sulfur causes excessive dehydrogenation of the binder. For this reason, binding materials such as coal and "green" coke which possess high softening temperatures cannot be used with sulfur for the purpose of the present invention. Suitable binder materials are coal tar pitch, coal depolymerization pitch and wood pitch having the indicated softening point.

Additionally it has been observed in the practice of the pressure baking process of interest that the number of pitch-bonded mixes which can be run without difficulty depends upon product weight. In the absence of sulfur in the pitch bonded mix, one or two 200 pound charges or sufficient to produce only four or five blocks 7 inches by 7 inches by 5 inches in size give off enough

condensate to cover the entire area near the mold. By contrast when using sulfur and pitch, over 3000, such blocks equivalent to more than 45,000 pounds of mix have been made without the need to clean the external parts of the press.

A large number of tests of the invention have been made. In such tests conventional mixes have been modified by the addition thereto of sulfur in accordance with the invention, and articles have been produced from the modified mixes. In typical tests, articles were produced from two basically similar mixes, both of which were used with sulfur and without sulfur. Each of the mixes was composed of "Calcined Ingredients," these being of petroleum coke of different particle sizes, and "Binder," the binder being a coal tar pitch having a melting point of 175° C. The composition of the mixes used in these tests is tabulated below:

TABLE I

| Mix No. | Mix Composition             |                             |                                        |        |
|---------|-----------------------------|-----------------------------|----------------------------------------|--------|
|         | Calcined Ingredients        |                             | Binder—Percent of Calcined Ingredients |        |
|         | Percent Coke A <sup>1</sup> | Percent Coke B <sup>1</sup> | Pitch                                  | Sulfur |
| I       | 25                          | 75                          | 15                                     | NH     |
| II      | 25                          | 75                          | 15                                     | 3      |
| III     | 50                          | 50                          | 15                                     | NH     |
| IV      | 50                          | 50                          | 15                                     | 3      |

<sup>1</sup> Particle sizes of: Coke A=0.015 inch to 0.03 inch, Coke B=55 percent through 200 mesh; 45 percent on 200 mesh (0.074 mm. openings).

In a series of tests conducted utilizing the mixes set forth in Table I, two different sizes of articles were produced. The first was a circular disc 1 1/4 inches in diameter by 5/8 inch thick. The second type of article produced was a brick measuring 9 inches by 4 1/2 inches by 2 1/2 inches. When mixes Nos. I and III were used (these mixes containing no sulfur), heavy, dark condensable fumes were produced. When mixes Nos. II and IV (that is, those containing sulfur) were used, under the same conditions, only light fumes which produced no condensate were formed. The apparent density of articles produced from the sulfur-containing mixes was only slightly greater than the apparent density of articles produced from the conventional mixes, indicating that most of the sulfur escaped during processing by combining the volatile constituents of the pitch binder. For example, the apparent density of a brick produced from mix No. I was 1.722 grams per cc., whereas a similar brick produced under similar conditions from mix No. II was 1.738 grams per cc. The longitudinal flexural strength of the brick produced from mix No. I was 3570 pounds per square inch, whereas that produced from Mix No. II was 3850 pounds per square inch.

What is claimed is:

1. In a process for making a formed carbon article from a mix consisting primarily of comminuted carbonaceous particles and fusible carbonaceous binder, said binder tending to evolve substances which condense on the apparatus used in said process, placing said mix in a mold, subjecting said mix within said mold to a high mechanical pressure to compress the same while passing an electrical current through said mix to heat the same to carbonization, the improvement which comprises providing in said mix in an amount ranging from 3 percent to 20 percent by weight of said binder material, said sulfur reacting with the substances evolved from said binder to form non-condensing materials whereby un-

wanted accumulation of condensable substances on said apparatus is avoided.

2. A process for making a formed carbon article comprising forming a mix comprising comminuted carbonaceous particles, sulfur, said sulfur being present in an amount ranging from 3 percent to 20 percent by weight of binder, and comminuted particles of a sulfur-reactive pitch binder having a melting point not in excess of 300° C.; enclosing said mix within the mold; subjecting said

mix within said mold to a high mechanical pressure to compress the same; while rapidly heating the compressed mixture to carbonization.

References Cited in the file of this patent

UNITED STATES PATENTS

1,017,483 Van Brunt ----- Feb. 13, 1912  
1,390,823 Sieurin ----- Sept. 13, 1921

UNITED STATES PATENT OFFICE  
CERTIFICATION OF CORRECTION

Patent No. 2,965,931

December 27, 1960

Lorne B. Alden et al.

It is hereby certified that error appears in the above numbered patent requiring correction and that the said Letters Patent should read as corrected below.

Column 2, line 69, after "mix" insert -- sulfur --.

Signed and sealed this 6th day of June 1961.

(SEAL)

Attest:

ERNEST W. SWIDER

Attesting Officer

DAVID L. LADD

Commissioner of Patents